

## UNITED STATES PATENT OFFICE.

CHARLES H. McALEER, OF DETROIT, MICHIGAN.

## CLEANSING AND POLISHING COMPOUND.

No Drawing.

Application filed December 12, 1924. Serial No. 755,368.

This invention relates to cleaning and polishing compounds, and the purpose of the invention is to provide a compound, the ingredients of which, in the application for 6 cleaning a surface, will leave it in a polished condition.

Heretofore, it has been commonly the practice in the cleaning of an automobile body and the metal parts thereof to first 10 apply an abrasive in the form of a compound that will clean the metal surfaces which requires to be washed and thereafter have applied thereto a wax or similar substance and polished. The purpose of this compound is 15 to secure both results in one application. The preferred proportion of the ingredients is as follows:

30 pounds double ground cream tripoli, 10 pounds powdered rottenstone, 2½ pounds 20 Kitigumi Japan wax, 2½ pounds double pressed stearic acid, 9 pounds kerosene, 2 pounds light rubbing oil.

These ingredients are thoroughly mixed together and packaged.

25 The tripoli and the rottenstone provide the abrasive elements of the composition while the stearic acid provides a bond or body. The kerosene and rubbing oil are used as a cleaner and as a lubricant for the 30 rubbing operation while the Japan wax is utilized for the purpose of producing a luster or polish. The abrasives are both finely powdered or ground so that no scratches apparent to the human eye are produced and 35 enables the surface to be scoured and in the rubbing operation for this scouring effect the Japan wax is deposited and polished. Subsequent to the application of the material in the cleaning and polishing operation, the 40 surface should be rubbed slightly with a dry cloth for the purpose of removing all particles of the compound and to produce a final luster. The light rubbing oil is a paraffine oil in which the paraffine has been 45 practically entirely removed. There is therefore no coagulate deposited that would destroy the final luster.

By this composition applied in the general manner indicated the surface to be cleaned 50 is polished and cleaned in the one operation and the surface is provided with a high luster that does not fade for a very considerable period of time.

The composition is very useful to manufacturers of metal automobile bodies, hoods, 55 fenders etc., in cleaning the bodies preparatory to transportation and maintains the metal parts free from rust and deterioration, and the customer sees the body in good condition and excellent appearance and is therefore in prime condition for application of 60 paint or enamel coats.

The composition is particularly beneficial in polishing finished automobile bodies whether painted, or lacquered surface, or the 65 now commonly used "Duco" finish. With such lacquer finishes the surface is not a perfectly smooth surface and, while the material of which the lacquer or finish is composed contains ingredients tending to produce a high polish does not produce the high 70 polish desired in that the surface is full of minute pits and scratches and therefore is not highly reflective of light. As above stated, my compound is useful in cleaning 75 and polishing such surfaces and my compound is designed to cut the surface to reduce the depth of the pits and to fill such pits as may remain and thus I secure a surface that is perfectly smooth and therefore 80 a highly light reflective surface.

The composition is found generally useful to the public in the cleaning and polishing of a finished painted automobile body or other article that requires cleaning and 85 polishing; is very simple to apply, and the resultant polished surface is secured by materially less effort than by any composition known to me that has heretofore been utilized.

90 It is further to be understood that some departure from the specific quantity of ingredients as specified may be made without departing from the spirit of the invention or materially varying the result to be attained. The broad feature of the invention resides in the inclusion of an ingredient producing a polish on the surface being cleaned by the rubbing operation and the ingredients as specified have been found by me to produce the most desirable result.

Having thus briefly described my invention, its utility and mode of operation, what I claim and desire to secure by Letters Patent of the United States is—

105 1. A cleansing and polishing compound

consisting of the following ingredients— namely, 30 pounds double ground cream tripoli, 10 pounds powdered rottenstone, 3½ pounds Kitigumi Japan wax, 2½ pounds double pressed stearic acid, 9 pounds kerosene and 2 pounds light rubbing oil.

2. A cleansing and polishing compound

consisting of a powdered abrasive, stearic acid, Japan wax, kerosene and a light rubbing oil.

In testimony whereof, I sign this specification.

CHARLES H. McALEER.